

[54] **METHOD FOR THE AFTERTREATMENT OF PAPER OR NONWOVEN FABRICS MADE OF INCOMPLETELY REGENERATED VISCOSE FIBERS**

[75] Inventor: **Yoshikazu Aoki, Otsu, Japan**

[73] Assignee: **Tachikawa Research Institute, Kyoto, Japan**

[22] Filed: **Dec. 7, 1973**

[21] Appl. No.: **214,969**

[52] U.S. Cl. .... **162/157 C; 8/152; 162/196**

[51] Int. Cl.<sup>2</sup> .... **D21H 5/12**

[58] **Field of Search** .... **162/157 C, 196; 264/181, 264/188, 195; 8/152, 156; 68/205 R, DIG. 5, 177, 178**

[56]

**References Cited**

**UNITED STATES PATENTS**

3,320,117 5/1967 Aoki et al. .... **162/157 C**  
3,608,109 9/1971 Fleissner et al. .... **68/DIG. 5**

*Primary Examiner*—S. Leon Bashore

*Assistant Examiner*—William F. Smith

[57]

**ABSTRACT**

In the process of making a paper product from incompletely regenerated viscose fibers, a washing step which includes the disposing of the washing net below the regeneration net a given distance and establishing a ratio of net speeds within a specified range.

**1 Claim, 2 Drawing Figures**



תינק 1



תינק 2



**METHOD FOR THE AFTERTREATMENT OF PAPER OR NONWOVEN FABRICS MADE OF INCOMPLETELY REGENERATED VISCOSE FIBERS**

This invention relates to the method for the useful and continuous aftertreatment of the wet sheet made of incompletely regenerated viscose fibers.

Paper or nonwoven fabrics made of incompletely regenerated viscose fibers is already well known, i.e., U.S. Pat. No. 3,320,117 and U.S. Pat. No. 3,553,078. In these processes incompletely regenerated viscose fibers are, after cutting in a suitable length, dispersed into water and a wet sheet is formed on a paper machine from the slurry. The wet sheet thus obtained is regenerated completely on a regeneration net, and after that in order to obtain the desired paper or nonwoven fabric, the wet sheet must be aftertreated or washed before drying, as in the conventional manufacture of viscose fibers. Desulphurization and bleaching of the sheet is then performed in the usual manner.

Generally speaking, there are two ways of washing a sheet, i.e., the fibrous sheet is washed successively on a washing net at the speed same as that of the paper machine, or the sheet is washed in a free state same as in the cellophane process. However, according to our experiments, it was found that these two methods are unsuitable to the treatment of the present wet sheet.

In the case of a heavy sheet the washing method used in the conventional cellophane process may be acceptable. However, in the treatment of a light sheet, the basic weight of which is less than 30 g/m<sup>2</sup>, difficulties are presented. In such a light sheet, the sheet was apt to be broken during the processing and, moreover, both edges of the sheet being apt to have an inside curl or fold. These problems precluded a smooth operation of the process.

On the other hand, if the running speed of the washing net is the same as that of the regeneration net, i.e., the paper machine speed, the process is preformed efficiently. However, in this case, the washing net must be dimensionally elongated in proportion to the increase in the paper machine speed in order to accomplish the desired washing because in this method, the washing net speed naturally must be increased with the increasing of the paper machine speed. It is a problem from a commercial viewpoint to use such a long net in the washing process.

The present invention is a proposal for solving the above-mentioned problems. It is no exaggeration to say that a successful washing method for a wet sheet formed of incompletely regenerated viscose fibers has been smoothly accomplished by the present invention notwithstanding the thickness of the wet sheets.

The present washing method is carried out originally by using a washing net. The running speed of the net is set to a certain speed less than that of the regeneration net. Under such a condition the wet sheet is shaken off from the regeneration net to the washing net placing the sheet in the folded state.

A better understanding of the invention may be had from the following description read in conjunction with the accompanying drawings, wherein:

FIG. 1 is a general view of the present washing method; and

FIG. 2 is an enlarged view showing the folded state of the sheet.

In FIG. 1, the wet sheet 1 on the regeneration net 2 is shaken off onto the washing net 4 keeping the folded state 3. Both nets are in the form of endless and porous or reticulated belts. In this case, the folded state of the sheet is determined by the speed ratio of both nets. The folded sheet is treated on the washing net by pouring the treating liquors from the washing trays 5. The washed sheet is sent to a dryer after being dehydrated by passing through press rolls 6, the speed of the dryer being the same as the speed of the paper machine.

In FIG. 2, the folded state of a sheet is shown. The fold in the sheet is a function of the speed ratio R of the washing net speed to the regeneration net speed and the distance A, the vertical distance between the nets. The smaller the speed ratio R and the larger the vertical distance A, the broader is the width B of the fold in the sheet.

According to our experiments, the value of R should be within the ratio 1/3 to 1/50. When R is larger than 1/3, the process loses its commercial value and when R is less than 1/50, the folded state of the sheet is not uniform and smooth operation is apt to be impaired.

On the other hand, the value of the vertical distance A should be set between 5 and 50. Only within such a range, is the uniform folding of the sheet possible.

After finishing the washing, the wet sheet is dehydrated after once again returning its running speed to the original speed, i.e., paper machine speed. In the present invention, the operation is smooth insofar as the folding of the sheet is uniformly effected. By adjusting R to between 1/3 and 1/50 and A to between 5 and 50 cm, it is possible to treat the sheet perfectly with a comparatively short machine at a fairly high speed.

**EXAMPLE 1**

After cutting in 10 mm length, incompletely regenerated viscose fibers were dispersed in water. A wet sheet was formed on a paper making wire net from the slurry at the speed of 50 m/min. After patterning the wet sheet, the sheet was regenerated completely on a regeneration net by pouring hot acid liquor containing 5 g/l of sulphuric acid at the same speed as that of the paper machine. After shaking off the wet sheet on the washing net, the washing treatments were done at three running speeds, i.e., 15, 5 and 1.2 m/min., respectively, for the washing net. In each case the vertical distance was set to 25 cm. The desulphurization was performed by the liquor containing 3 g/l of caustic soda at the temperature of 80°C, and the bleaching by the sodium hypochlorite liquor containing 1 g/l of available chlorine at the temperature of 20°C.

In order to estimate the effect of the present treatment, the reducible sulphur content of the product sheets was measured quantitatively. The results are shown in the following table.

**TABLE**

| Running Speed(m/min)<br>Regeneration<br>Net | Washing<br>Net | Speed Ratio<br>(R) | Reducible Sulphur<br>of the Product (%) |
|---------------------------------------------|----------------|--------------------|-----------------------------------------|
| 50                                          | 15             | 3/10               | 0.006                                   |
| 50                                          | 5              | 1/10               | 0.005                                   |
| 50                                          | 1.2            | 1.2/50             | 0.005                                   |

It is clear from the Table that the effect of the present washing is constant in the wide range of the speed ratio R.

What is claimed is:

1. In a process for manufacturing paper or nonwoven fabrics from incompletely regenerated viscose fibers which have been dispersed in water to form a slurry and subsequently formed into a wet sheet on a paper making machine, completely regenerating the fibers of the sheet on a regeneration net traveling the same running speed as said paper making machine, the improvement comprising the steps of desulphurizing and bleaching the completely regenerated sheet with desulphurizing

10

and bleaching treating liquors respectively on a washing net having a running speed of from 1/3 to 1/50 of the speed of said regeneration net, the vertical distance between the regeneration net and the washing net being from 5 to 50 centimeters, and drying the desulphurized and bleached sheet in a drier, said drier including press rolls having the same running speed as said regeneration net.

\* \* \* \* \*

15

20

25

30

35

40

45

50

55

60

65